

Patented Apr. 6, 1943

2,315,507

UNITED STATES PATENT OFFICE

2,315,507

COPPER-BASE ALLOY

Reginald S. Dean and Clarence T. Anderson, Salt Lake City, Utah, assignors to Chicago Development Company, Chicago, Ill., a corporation of Illinois

No Drawing. Application October 1, 1941,  
Serial No. 413,160

5 Claims. (Cl. 75—161)

Our invention relates to the preparation of alloys having good corrosion resistance under atmospheric conditions.

The alloys to which our invention relates are copper-base alloys containing from about 2% to about 25% manganese, from about 2% to about 20% chromium, from about 2% to about 25% iron, balance substantially all copper. Preferably, the alloys of our invention contain from about 70% to about 90% copper, balance consist-

ing of manganese, chromium, and iron, each in percentages of at least about 2%.

The following table shows a number of illustrative alloys made in accordance with our present invention and wherein various of the properties of the said alloys are listed. In the table, Rc means Rockwell C scale; C. W. means cold worked; Q means quenched; and S. C. means slow cooled.

| No. | Comp.                               | Hardness as cast | Hardness C. W.<br>.251 | Q 450° C. | Q 550° C. | Q 650° C. | Coefficient of expansion | Resistivity                                                         | Corrosion test 10% NaCl intermittent    | Corrosion test 5% H <sub>2</sub> SO <sub>4</sub> intermittent |
|-----|-------------------------------------|------------------|------------------------|-----------|-----------|-----------|--------------------------|---------------------------------------------------------------------|-----------------------------------------|---------------------------------------------------------------|
| 1   | Mn 2.5<br>Cr 2.5<br>Cu 90<br>Fe 5   | Rc —46           | Rc —15                 | Rc —19    | Rc —17    | Rc —32    | 14.74×10 <sup>-6</sup>   | C. W. 17.0×10 <sup>-6</sup><br>S. C. 900° C. 10.2×10 <sup>-6</sup>  | Slight rusting                          | Pickle only.                                                  |
| 2   | Mn 2.5<br>Cr 2.5<br>Cu 85<br>Fe 10  | Rc —42           | Rc —7                  | Rc —12    | Rc —16    | Rc —24    | 13.80×10 <sup>-6</sup>   | C. W. 18.4×10 <sup>-6</sup><br>S. C. 900° C. 10.8×10 <sup>-6</sup>  | Darkening of surface.                   | Pickle only.                                                  |
| 3   | Mn 5<br>Cr 5<br>Cu 85<br>Fe 5       | Rc —42           | Rc —1                  | Rc —9     | Rc —10    | Rc —25    | 14.16×10 <sup>-6</sup>   | C. W. 24.7×10 <sup>-6</sup><br>S. C. 900° C. 19.4×10 <sup>-6</sup>  | Darkening of surface.                   | Pickle only.                                                  |
| 4   | Mn 5<br>Cr 5<br>Cu 80<br>Fe 10      | Rc —27           | Rc 0                   | Rc —3     | Rc —6     | Rc —25    | 13.38×10 <sup>-6</sup>   | C. W. 31.6×10 <sup>-6</sup><br>S. C. 900° C. 25.4×10 <sup>-6</sup>  | Darkening of surface.                   | Pickle only.                                                  |
| 5   | Mn 2.5<br>Cr 2.5<br>Cu 80<br>Fe 15  | Rc —32           | Rc +1                  | Rc —5     | Rc —5     | Rc —19    | 13.74×10 <sup>-6</sup>   | C. W. 22.0×10 <sup>-6</sup><br>S. C. 900° C. 15.1×10 <sup>-6</sup>  | Rusted at surface cracks.               | Pickle only.                                                  |
| 6   | Mn 2.5<br>Cr 2.5<br>Cu 75<br>Fe 20  | Rc —24           | Rc +3                  | Rc 0      | Rc —7     | Rc —22    | 12.70×10 <sup>-6</sup>   | C. W. 22.7×10 <sup>-6</sup><br>S. C. 900° C. 14.6×10 <sup>-6</sup>  | Heavy rusting of surface.               | Pickle only.                                                  |
| 7   | Mn 5<br>Cr 5<br>Cu 75<br>Fe 15      | Rc —27           | Rc +2                  | Rc —3     | Rc —8     | Rc —22    | 13.05×10 <sup>-6</sup>   | C. W. 29.6×10 <sup>-6</sup><br>S. C. 900° C. 22.3×10 <sup>-6</sup>  | Darkening of surface.                   | Pickle only.                                                  |
| 8   | Mn 7.5<br>Cr 7.5<br>Cu 75<br>Fe 10  | Rc —26           | Rc +4                  | Rc +2     | Rc —3     | Rc —20    | 12.72×10 <sup>-6</sup>   | C. W. 37.8×10 <sup>-6</sup><br>S. C. 900° C. 31.6×10 <sup>-6</sup>  | Darkening of surface.                   | Pickle only.                                                  |
| 9   | Mn 10<br>Cr 10<br>Cu 75<br>Fe 5     | Rc —24           | Rc +11                 | Rc +7     | Rc +1     | Rc —13    | 13.40×10 <sup>-6</sup>   | C. W. 44.1×10 <sup>-6</sup><br>S. C. 900° C. 38.2×10 <sup>-6</sup>  | Darkening of surface.                   | Pickle only.                                                  |
| 10  | Mn 2.5<br>Cr 2.5<br>Cu 70<br>Fe 25  | Rc —12           | Rc +1                  | Rc +4     | Rc —2     | Rc —16    | 12.30×10 <sup>-6</sup>   | C. W. 24.4×10 <sup>-6</sup><br>S. C. 900° C. 15.84×10 <sup>-6</sup> | Heavy rusting of surface.               | Pickle only.                                                  |
| 11  | Mn 5<br>Cr 5<br>Cu 70<br>Fe 20      | Rc —24           | Rc +3                  | Rc —1     | Rc —6     | Rc —22    | 12.54×10 <sup>-6</sup>   | C. W. 32.4×10 <sup>-6</sup><br>S. C. 900° C. 25.2×10 <sup>-6</sup>  | Slight rusting at small surface cracks. | Pickle only.                                                  |
| 12  | Mn 7.5<br>Cr 7.5<br>Cu 70<br>Fe 15  | Rc —22           | Rc +9                  | Rc +2     | Rc —1     | Rc —12    | 13.71×10 <sup>-6</sup>   | C. W. 46.1×10 <sup>-6</sup><br>S. C. 900° C. 42.3×10 <sup>-6</sup>  | Slight rusting at small surface cracks. | Pickle only.                                                  |
| 13  | Mn 10<br>Cr 10<br>Cu 70<br>Fe 10    | Rc —21           | Rc +7                  | Rc —1     | Rc 0      | Rc —23    | 12.75×10 <sup>-6</sup>   | C. W. 39.5×10 <sup>-6</sup><br>S. C. 900° C. 32.9×10 <sup>-6</sup>  | Darkening of surface.                   | Pickle only.                                                  |
| 14  | Mn 12.5<br>Cr 12.5<br>Cu 70<br>Fe 5 | Rc —19           | Rc +11                 | Rc +11    | Rc +1     | Rc —9     | 13.71×10 <sup>-6</sup>   | C. W. 55.0×10 <sup>-6</sup><br>S. C. 900° C. 49.6×10 <sup>-6</sup>  | Darkening of surface.                   | Pickle only.                                                  |

Alloy No. 3, for example, listed in the above table, made from highly pure metals such as are obtained by electrolytic refining, is highly ductile and may be rolled into sheets or drawn into a wire or a rod. When such sheet, wire or rod is annealed at a temperature of about 750 degrees C., it has a tensile strength of approximately 45,000 pounds per square inch. On cold working, a tensile strength of about 75,000 pounds per square inch may be obtained. By intermediate amounts of rolling or by annealing at temperatures below 650 degrees C., any desired intermediate degree of hardness may be obtained. The modulus of elasticity of the alloy is  $22 \times 10^6$  pounds per square inch. The alloy shows only a slight darkening in an extended alternate immersion test in a 10% sodium chloride solution, and is not attacked in a 5% sulphuric acid solution.

All of the alloys of our invention possess fairly good resistance to atmospheric corrosion. Those of the alloys which contain more than 15% iron, however, undergo some rusting by extended alternate immersion in 10% sodium chloride solution. Slight rusting also occurs with alloys containing a low as 5% iron where the manganese content is approximately 2.5%. This rusting, however, in connection with the latter alloy, is completely overcome by the employment of 5% manganese and 5% chromium. The preferred embodiments of our invention, therefore, where alloys are desired which are resistant to corrosion in salt water, encompass alloys containing from about 5% to about 15% manganese, from about 5% to about 15% chromium, from about 5% to about 15% iron, balance substantially all copper.

In the above table, it will be noted that we have expressed the hardness of the alloys, in various conditions, on the Rockwell C scale. For the purpose of correlating the hardness with the tensile strength, it may be pointed out that a hardness of Rockwell C -30 corresponds to a tensile strength of approximately 45,000 pounds per square inch, a hardness of Rockwell C zero corresponds to a tensile strength of approximately 75,000 pounds per square inch, and a hardness of Rockwell C 10 corresponds to a tensile strength of approximately 95,000 pounds per square inch. On this basis, it will be seen that an alloy containing 75% copper, 10% manganese, 10% chromium, and 5% iron (No. 9 of the above table) may be cold rolled to produce an alloy having a tensile strength of 95,000 pounds per square inch. The electrical resistance of such an alloy is  $44.1 \times 10^{-6}$  ohms/cm.<sup>2</sup>

While the alloys of our invention have, generally speaking, many properties similar to those of nickel silvers, they have, in addition, certain advantages over nickel silvers in that, among other things, many of them possess a wider range of work hardening properties as well as a wider range of electrical resistance.

As we have indicated hereinabove, we prefer to employ highly pure metals in the preparation of the alloys of our present invention. We prefer, particularly, to utilize metals produced electrolytically. In the case of manganese, for best results the said metal should have a purity of at least 99.0%, electrolytic manganese of a purity of 99.9% being especially satisfactory.

In the light of the various properties of the alloys which have been described hereinabove, it will be apparent to those versed in the art that the said alloys may be utilized in various ways and for various purposes in the industrial and engineering fields. Illustrative uses of the alloys of our invention are for the preparation of springs, ratchets, pawls, electrical resistance wire, condenser tubes and other equipment requiring resistance to corrosion by steam, decorative articles, and for other purposes to which nickel silvers, monel metal, and other alloys having a high nickel content are usually put.

What we claim as new and desire to protect by Letters Patent of the United States is:

1. Alloys, having good corrosion resisting properties, containing about 2% to about 25% manganese, about 2% to about 20% chromium, about 2% to about 25% iron, balance substantially all copper.
2. Alloys, having good resistance to corrosion, containing about 5% to about 15% manganese, about 5% to about 15% iron, balance substantially all copper.
3. Alloys having good corrosion resisting properties containing about 2% to about 25% manganese, about 2% to about 20% chromium, about 2% to about 25% iron, balance copper, the copper constituting from 70% to 90% of the alloys.
4. Alloys, having good corrosion resisting properties, containing about 2% to about 25% electrolytic manganese having a purity of at least 99.9%, about 2% to about 20% chromium, about 5% to about 15% iron, balance substantially all copper.
5. Alloys, having good resistance to corrosion, containing about 5% to about 10% manganese, about 5% to about 10% chromium, about 5% to about 10% iron, balance substantially all copper.

REGINALD S. DEAN.  
CLARENCE T. ANDERSON.